

## UNITED STATES PATENT OFFICE

2,083,456

## MANUFACTURE OF COILED-COIL FILAMENTS FOR ELECTRIC INCANDESCENT LAMPS AND SIMILAR DEVICES

Reginald Edward Leeds, Middlesex, England, assignor to General Electric Company, a corporation of New York

No Drawing. Application January 7, 1937, Serial No. 119,527. In Great Britain December 11, 1935

6 Claims. (Cl. 175—40)

This invention relates to the manufacture of coiled-coil filaments for electric incandescent lamps and similar devices.

Coiled-coil filaments are described in British patent specification No. 6,439 of 1914; but no detailed directions are given concerning their manufacture; in particular no heat treatment of the wire at any stage of the coiling is prescribed. In several later specifications heat treatment 10 after the winding of the secondary helix is prescribed at a temperature considerably exceeding 1000° C. Part at least of the object of this treatment is said to be the improvement of the stability of the filament, so that it will not sag seriously when maintained at the operating temperature. The increased stability is sometimes thought to be associated with the growth of long crystals. It appears to be believed very widely at the present time, that heating the secondary 20 helix to a temperature considerably exceeding 1000° C. is essential to obtaining a stability sufficient for commercial purposes. So far as I am aware, such a heat treatment is applied in all commercial processes for making coiled-coil filaments practiced at the present time.

I have found that in suitable circumstances a stability of the filament sufficient for commercial lamps can be obtained without heating the secondary helix to any temperature above 1000° C. Sometimes the required stability can be obtained without any heating of the wire during coiling, that is to say at any stage between the cessation of wire-drawing and the mounting of the coiled-coil filament on its final supports in the lamp. In other circumstances heat treatment 30 may be necessary either before the secondary helix is wound or after it is wound or both; but it may still be possible to obtain the required stability without raising the temperature of the wire after the secondary helix is wound to above 1000° C. If the secondary helix has not to be heated, manufacture may be simplified and cheapened; thus it is not necessary to use the expensive molybdenum mandrels for the secondary helix which are necessary if (as in some known processes) the secondary helix is heated on its mandrel to 1500° C.

In order that these results may be achieved, 50 two conditions must be fulfilled. The first is that the wire must be suitable. One of the necessary properties is ability to grow stable long crystals almost instantaneously when the completed filament is first heated in the lamp to or near to its operating temperature. Long crystals

means those whose length is not less than the diameter of the wire.

It will be appreciated by those skilled in the art that it is impossible to prescribe with certainty all the necessary preparations or that set 5 of them which is sufficient. It is well known that, in all filament manufacture, behavior in the lamp is the only safe criterion, and that the most careful description of the method of preparation or of tests to be applied (not simulating 10 actual use) does not suffice to ensure that all wires will be of the desired quality. On the other hand, wires that are suitable for the manufacture according to the invention may be expected to be found in the stock of any well-15 equipped maker of tungsten wire for filaments.

The methods of preparation which, in my experiments, have yielded suitable wire are (a) the well-known modern silicated process, which is a development of that described in British patent 20 specification No. 155,851, and (b) a process of subjecting a wire containing about three-fourths 25 per cent of thoria to a thermo-mechanical process of the kind described in British patent specification No. 183,118. It can be stated definitely 25 that no method of preparation known at the date of the aforesaid British patent specification No. 6,439 of 1914 will yield suitable wire.

Concerning the properties that the resulting 30 wire should possess, it may be said that they are generally those recognized as favorable in the manufacture of coiled-coil filaments by known methods; in particular, the greater the tendency 35 of the wire to grow long crystals rapidly when coiled in the usual manner, the greater, in general, will be the tendency to grow long crystals rapidly when coiled according to the invention.

The second condition aforesaid is that the 40 strains produced in the wire by the winding of the primary helix shall be at least partially released before the secondary helix is wound. These strains may be released, for example, by dissolving out the primary mandrel or by heating the primary helix on a mandrel of molybdenum 45 to a sufficiently high temperature, for example, 1600° C.

According to the invention, a process of manufacturing coiled-coil filaments for electric incandescent lamps comprises the following steps in the following order: (1) winding on a mandrel a 50 tungsten wire capable of growing long crystals almost instantaneously when first heated to the operating temperature, so as to produce a primary helix, (2) releasing part at least of the strain in the wire generated by the said winding, 55

(3) winding the primary helix on a mandrel so as to form a secondary helix, (4) removing the secondary mandrel, wherein the said wire, between the beginning of step (3) and the end of step (4) never rises to a temperature greater than 1000° C.

In steps (1) and (3) the diameter of the mandrel must be so small that a sufficient permanent set shall be given to the wire. A permanent set 10 may be encouraged in step (3) by heating the tungsten wire to a temperature below 1000° C., e. g. 400° to 800° C. In suitable conditions a sufficient set may be obtained even if the diameter of the mandrel is as great as four times the 15 diameter of the wire in both steps. If in step (2) the strain is released by dissolving out the mandrel, the primary helix must be subjected to a small suitably chosen tension in step (3).

Three processes according to the invention 20 will now be described by way of example. In all of them the tungsten wire, which serves as starting material, was a silicated wire of the type described in the above-mentioned British Patent 155,851 and known to give excellent coiled-coil filaments by known process.

In the first process, the original wire was 0.031 25 mm. in diameter. It was coiled into a helix 80 mms. long with a pitch of 0.0396 mm. on a molybdenum mandrel 0.12 mm. in diameter. This 30 primary mandrel was dissolved out. The secondary helix was formed by winding this primary helix in 137 turns on a mandrel again 0.12 mm. in diameter with a pitch of 0.182 mm., that is to say, with the turns touching. During this secondary winding the primary helix was stretched 35 so that its pitch became 0.0538 mm. The secondary helix was heated to 400° C. for two minutes to encourage a permanent set; after removal 40 of the secondary mandrel the pitch of the secondary helix was 0.357 mm. and the number of turns 100.

The second process was generally similar, but the dimensions were changed and there was no heating in step (3) referred to above. The original wire was 0.024 mm. diameter; the primary 45 mandrel 0.045 mm. diameter, the primary pitch 0.0293 mm., the length of the primary helix 108 mm. The secondary mandrel was 0.12 mm. in diameter, the pitch of the primary helix during 50 winding of the secondary helix was 0.0333 mm., the secondary pitch 0.093 mm. (turns touching), the number of secondary turns 217. After removal of the secondary mandrel, the secondary pitch was 0.196 mm. and the number of turns 157.

In the third process, the original wire was 0.024 mm. diameter, the primary molybdenum 55 mandrel 0.045 mm., the primary pitch 0.040 mm. The primary helix was heated on the mandrel to 1500° C. for twelve seconds, but the mandrel was not removed. The secondary mandrel was 0.210 mm. diameter, the pitch 0.155 (turns not touching), the number of turns 155. After the winding 60 of the secondary helix, the wire was heated to 750° C. for thirty seconds. After removal of the mandrels, the pitch of the secondary helix was 0.176 mm.; the number of turns 136.

What I claim as new and desire to secure by Letters Patent of the United States is:

1. The process of manufacturing coiled-coil 70 filaments for electric incandescent lamps which comprises winding on a mandrel a tungsten wire which grows long crystals almost instantaneously when first heated to the operating temperature

in the lamp, so as to produce a primary helix, releasing at least part of the strain in the wire produced by the winding, winding the primary helix on a secondary mandrel so as to form a secondary helix, heating the secondary helix to a temperature maintained below 1000° C., and then removing the secondary mandrel.

2. The process of manufacturing coiled-coil 10 filaments for electric incandescent lamps which comprises winding on a mandrel a tungsten wire which grows long crystals almost instantaneously 15 when first heated to the operating temperature in the lamp, so as to produce a primary helix, removing said mandrel to release at least part of the strain in the wire produced by the winding, winding the primary helix on a secondary mandrel so as to form a secondary helix, heating the secondary helix to a temperature maintained below 1000° C., and then removing the secondary 20 mandrel.

3. The process of manufacturing coiled-coil 25 filaments for electric incandescent lamps which comprises winding on a mandrel a tungsten wire which grows long crystals almost instantaneously 30 when first heated to the operating temperature in the lamp, so as to produce a primary helix, heating the wire to a temperature of at least 1500° C. to release at least part of the strain in the wire produced by the winding, winding the primary helix on a secondary mandrel so as to 35 form a secondary helix, heating the secondary helix to a temperature maintained below 1000° C., and then removing the secondary mandrel.

4. The process of manufacturing coiled-coil 40 filaments for electric incandescent lamps which 45 comprises winding on a mandrel a tungsten wire which grows long crystals almost instantaneously when first heated to the operating temperature in the lamp, so as to produce a primary helix, releasing at least part of the strain in the wire produced by the winding, winding the primary helix on a secondary mandrel so as to form a secondary helix, heating the secondary helix to a temperature of between 400° C. and 800° C., and then removing the secondary mandrel.

5. The process of manufacturing coiled-coil 50 filaments for electric incandescent lamps which comprises winding on a mandrel a tungsten wire which grows long crystals almost instantaneously 55 when first heated to the operating temperature in the lamp, so as to produce a primary helix, removing said mandrel to release at least part of the strain in the wire produced by the winding, winding the primary helix on a secondary mandrel so as to form a secondary helix, heating the secondary 60 helix to a temperature of between 400° C. and 800° C., and then removing the secondary mandrel.

6. The process of manufacturing coiled-coil 65 filaments for electric incandescent lamps which 70 comprises winding on a mandrel a tungsten wire which grows long crystals almost instantaneously when first heated to the operating temperature in the lamp, so as to produce a primary helix, heating the wire to a temperature of at least 65 1500° C. to release at least part of the strain in the wire produced by the winding, winding the primary helix on a secondary mandrel so as to form a secondary helix, heating the secondary 75 helix to a temperature of between 400° C. and 800° C., and then removing the secondary mandrel.

REGINALD EDWARD LEEDS.